

1

2,832,739

## UREIDO THICKENED GREASES

Edward A. Swakon, Hammond, Ind., assignor to Standard Oil Company, Chicago, Ill., a corporation of Indiana

No Drawing. Application June 13, 1955  
Serial No. 515,257

13 Claims. (Cl. 252—49.6)

The present invention relates to novel lubricant greases and to the method of preparing same. More particularly, it relates to novel greases comprising a lubricant vehicle thickened with certain high melting ureido compounds. Greases of this type have demonstrated exceptional stability at elevated temperatures.

As lubricants are required to perform at higher and higher temperatures because of increased speeds of engines and machines, the advent of jet propulsion, atomic energy as a source of power, etc., it has become increasingly difficult to prepare greases fulfilling the requirements of such lubricants. In attempting to provide such greases, the art has progressed from the use of petroleum lubricant vehicles thickened with metal soaps of long chain fatty acids, e. g. lithium hydroxy-stearate, to more thermally stable synthetic lubricating oils such as the aliphatic diesters of dicarboxylic acids, silicone polymers, etc., thickened with such soaps or inorganic materials such as silica gels. The progress of thickener research has not in general, however, kept pace with the development of lubricant vehicles. And at temperatures as high as 400° to 450° F. there are few if any greases available which will retain their consistency and lubricity for any substantial period of time.

In recent years various synthetic lubricant vehicles, e. g. the silicones, fluorocarbons, etc., have been found to be potentially valuable for use in greases employed at very high temperatures because of their thermal stability and relatively low volatility. Unless, however, a thickener having substantially the same degree of thermal stability is available to produce a grease from such an oil, they are of little use.

It is a primary object of the present invention to provide lubricant greases which are stable and give excellent lubrication at elevated temperatures. A further object is to provide a readily producible series of greases embodying a novel class of thickening agents capable of yielding lubricants particularly suitable for use at temperatures of from about 250° F. to about 450° F. A particular object of the present invention is to provide greases which are effective lubricants at temperatures as high as about 450° F. for substantial periods of time. These and additional objects will be apparent from the following detailed description.

Copending Swakon and Brannen application for Letters Patent S. N. 318,321, filed November 1, 1952, now U. S. 2,710,839, discloses and claims certain very high melting aromatic ureas, diureas, amides, and diamides, all of which contain at least one



wherein R is an aryl radical; and which are referred to broadly as aryl carbamyl compounds, as thickeners of silicone polymer oils, as well as other known lubricant vehicles, to produce greases which are stable and display excellent lubricant properties over a wide range of temperatures. Whereas silicone polymer oils are particularly

2

preferred for use in greases employed at temperatures as high as about 450° F., other lubricant vehicles, either natural or synthetic, may also be thickened with these materials to produce greases of particular utility over a wide range of temperatures.

In copending Swakon and Brannen application for Letters Patent S. N. 393,010, filed November 18, 1953, now U. S. 2,710,840, greases prepared with thickeners comprising mixtures of at least two different aryl substituted ureas and/or diureas are described and claimed. Thus, in accordance with the invention described in said application, mixtures of aryl substituted ureas prepared by reacting (1) at least two different aryl monoisocyanates with at least one aryl amine (mono- or di-amine) or (2) at least two different aryl monoamines with at least one aryl isocyanate (mono- or diisocyanate).

It has now been found that grease compositions exhibiting good rheological properties, having high thermal stability and possessing high dropping points and/or no melt characteristics can be obtained by thickening a suitable oleaginous lubricant vehicle with from about 2% to about 50% and preferably from about 5% to about 40%, by weight, of a ureido compound having the general formula

25  $Z—R—NH—CO—NH—R'—(NH—CO—NH—R'')_xZ'$   
in which Z and Z' are terminal reactive radicals selected from the group consisting of  $—NH_2$  and  $—NCO$  radicals and mixtures thereof, x is an integer 0 to 5, and R, R', and R'' are the same or different organic radicals selected from the group consisting of an alkylene radical, a substituted alkylene radical, an arylene radical, a substituted arylene radical, heterocyclic radical and mixtures thereof. The substituted alkylene and arylene radicals can contain substituents such as, by way of example, alkyl, aryl, hydroxy, carboxy, halogen, nitro, carboalkoxy, alkoxy, cyano and other groups. The alkylene and substituted alkylene groups are further characterized as straight and/or branched chain radicals having from 1 to about 30 carbon. The arylene and substituted arylene radicals can be mononuclear and/or polynuclear such as phenylene, biphenylene, naphthylene and anthrylene radicals.

The ureido compounds are readily prepared by heating a mixture of the polyamine and the polyisocyanate in equivalent weight ratios of from 1:x to x:1 where x can be a number ranging from 2 to 4, and preferably in the equivalent weight ratio of 1:1, at a temperature within the range of room temperature (about 70° F.) to about 350° F. For example, when diamines and diisocyanates are the reactants the equivalent weight ratio can be varied from 1:2 to 2:1, while when triamines and triisocyanates are the reactants the equivalent weight ratio can be varied from 1:3 to 3:1. One or more polyamines can be reacted with one or more polyisocyanates to give mixed polyureido compounds. As indicated in the general formula above, the herein described ureido compounds can have one amino- and one isocyanato-terminal radical or both terminal radicals can be the same, i. e. either amino radicals or isocyanato radicals depending upon the equivalent weight ratio of the reactants used. Thus when the polyamine and the polyisocyanate are used in the equivalent weight ratio of 1:1, the resultant reaction products will contain predominantly ureido compounds having amino and isocyanato terminal radicals; when the reaction mixture contains an excess of the polyamine, the resultant reaction products will contain ureido compounds the terminal groups of which are predominantly amino radicals, and when the reaction mixture contains an excess of the polyisocyanate, reaction products containing ureido compounds having predominantly isocyanato-terminal groups will be obtained.

When the polyamine is a diamine and the polyisocyanate is a diisocyanate the resultant polyureido compounds are linear. However, if one or more of the reactants is a polyamine greater than a diamine, for example, a triamine, such as 1,3,5-triaminobenzene, or the polyisocyanate is greater than a diisocyanate, for example, a triisocyanate, such as, 1,3,5-benzenetriisocyanate, cross-linked polyureido compounds can be formed. The free terminal amino and isocyanate groups can be reacted further with other reactive compounds such as monoamines, isocyanates, water, etc. Thus, for example, when water is added to a polyureido compound, the terminal —NCO group can be transformed to an amino group (—NH<sub>2</sub>); or, if, for example, phenyl isocyanate is added, some of the terminal free amines are blocked and transformed to phenyl ureido groups.

Examples of suitable polyisocyanates which can be employed in accordance herewith are tolylene diisocyanate, p,p'-diisocyanate biphenyl, 1,4-diisocyanato-benzene, p,p'-diisocyanato-diphenylmethane, 1,6-diisocyanato hexane, 1,12-diisocyanato dodecane, 1,3,5-benzene triisocyanate, naphthylene diisocyanate, bitolylen diisocyanate, tris-p-isocyanatophenyl-methane.

Examples of suitable polyamines are benzidine, p-phenylene-diamine, o-phenylenediamine, m-phenylenediamine, o-tolidine, triamino-benzene, 1,6-diaminohexane, 1,10-diaminodecane, 1,3-diaminopropane, dialkylenetriamine, trialkylenetetramine, ethylenediamine, xylylenediamine, tolylenediamine, dimethyl-p-phenylenediamine, etc.

Polyureido compounds of the type herein described can be prepared by the reaction of water on a polyisocyanate in accordance with the probable reaction as illustrated by the following equations:



where the R represents organic radicals as above defined. (While the reaction of the polyamine and the polyisocyanate in a mole ratio of 1:1 will give ureido compounds having amino- and isocyanato-terminal radicals, in the above preparation wherein the polyamine is first obtained by the hydrolysis of the polyisocyanate, excess water present as indicated for the last reaction, hydrolyzes the isocyanato-terminal radical of the final product to an amino-radical.) The above reaction is illustrated by the following specific example using bitolylen diisocyanate:



The resultant o-tolidine (III) is reacted with additional bitolylen diisocyanate in the presence of water to give a polymer such as



The general structural formulae of illustrative ureido compounds of the type herein described are:

- (a)  $\text{H}_2\text{N}-\text{Ar}-\text{NH}-\text{CO}-\text{NH}-\text{Ar}-\text{NCO}$
- (b)  $\text{H}_2\text{N}-\text{Ar}-\text{NH}-\text{CO}-\text{NH}-\text{Ar}-$   
5  $\text{NH}-\text{CO}-\text{NH}-\text{Ar}-\text{NCO}$
- (c)  $\text{H}_2\text{N}-\text{Ar}-\text{NH}-\text{CO}-\text{NH}-\text{Ar}'-$   
10  $\text{NH}-\text{CO}-\text{NH}-\text{Ar}-\text{NCO}$
- (d)  $\text{H}_2\text{N}-\text{Ar}-\text{NH}-\text{CO}-\text{NH}-\text{Ar}'-\text{NH}-$   
15  $\text{CO}-\text{NH}-\text{Ar}-\text{NH}-\text{CO}-\text{NH}-\text{Ar}'-\text{NCO}$
- (e)  $\text{H}_2\text{NR}-\text{NH}-\text{CO}-\text{NH}-\text{Ar}-\text{NCO}$
- (f)  $\text{H}_2\text{N}-\text{Ar}-\text{NH}-\text{CO}-\text{NH}-\text{R}-\text{NCO}$
- (g)  $\text{H}_2\text{N}-\text{R}-\text{NH}-\text{CO}-\text{NH}-\text{R}-$   
15  $\text{NH}-\text{CO}-\text{NH}-\text{R}-\text{NCO}$
- (h)  $\text{H}_2\text{N}-\text{R}-\text{NH}-\text{CO}-\text{NH}-\text{R}-$   
20  $\text{NH}-\text{CO}-\text{NH}-\text{Ar}-\text{NCO}$
- (i)  $\text{H}_2\text{N}-\text{Ar}-\text{NH}-\text{CO}-\text{NH}-\text{R}'-\text{NH}-\text{CO}-$   
25  $\text{NH}-\text{Ar}-\text{NH}-\text{CO}-\text{NH}-\text{R}''-\text{NCO}$

wherein Ar represents a phenylene radical, Ar' represents a biphenylene radical, R represents a  $(\text{CH}_2)_{18}$  alkylene radical, R' represents a  $(\text{CH}_2)_6$  alkylene radical and R'' represents  $(\text{CH}_2)_{16}$  alkylene radical.

While the above formulae are illustrative of ureido compounds containing an amino- and an isocyanato-terminal group, the present invention is not limited to such ureido compounds, but includes ureido compounds having amino-terminal groups or isocyanato-terminal groups, as shown by the general formulae given above.

Oleaginous lubricant vehicles which can be thickened 30 with the herein described polyureido compounds to form greases of the present invention can be silicone polymer oils, mineral lubricating oils, synthetic hydrocarbon lubricating oils, synthetic lubricating oil-such as polyalkylene glycols and their derivatives, high molecular weight esters of dicarboxylic acids, polyfluoro derivatives of organic compounds such as the trifluorovinyl chloride polymers known as "Fluorolube" (made by Hooker Chemical Company) and the trifluorochloroethylene polymers, known as "Kel-F-40" (made by The M. W. Kellogg Company), and other lubricant vehicles.

The silicone polymer oils which may be employed in accordance with the present invention are those falling substantially within the lubricating oil viscosity range. In general, such oils have the following unit structure:



wherein R and R' represent substituted or unsubstituted alkyl, aryl, alkylaryl, arylalkyl or cycloalkyl radicals. Such compounds may be produced by well-known methods, e. g. the hydrolysis or dialkylchlorosilanes or dialkyl-diethoxysilanes with a suitable chain stopper, e. g. a tri-substituted mono-chlorosilane. For purposes of the present invention, those polymers which are high boiling liquids within the lubricating oil viscosity range are suitable, these generally possessing a viscosity at 100° F. which is within the range of from about 25 to about 3500

60 S. S. U. It is preferred, for purposes hereof, to employ such oils as have a viscosity at 100° F. of from about 100 S. S. U. to about 1250 S. S. U. Such products are generally colorless and inert, have a very low volatility and undergo relatively slight change in viscosity for a given change in temperature. Relatively common oils of this type are dimethylsilicone polymer, phenylmethylsilicone polymer, chlorophenylmethylsilicone polymer, etc., it being preferred to employ either the phenylmethylsilicone or the chlorophenylmethylsilicone polymer in accordance 65 herewith. Methods of preparing such compounds are

taught in numerous patents, e. g. U. S. 2,410,346, U. S. 2,456,496, and in the literature such as "Chemistry of the Silicones," by Rochow, page 61, et seq. A particularly desirable phenylmethylsilicone polymer for use in accordance with the present invention is Dow-Corning 550 Silicone Fluid, a product of Dow-Corning, Inc., which has a Saybolt Universal viscosity at 100° F. of about 300 to about 400 seconds. Another suitable silicone polymer is a chlorophenylmethylsilicone marketed as GE 81406 by General Electric Company.

Other oleaginous vehicles which may be employed here-with are, for example, mineral oils in the lubricating oil viscosity range, i. e. from about 50 S. S. U. at 100° F. to about 300 S. S. U. at 210° F. These mineral oils are preferably solvent extracted, to substantially remove the low V. I. constituents, e. g. aromatics, with phenol, furfural, B,B'-dichlorodiethylether (Chlorex), liquid SO<sub>2</sub>, nitrobenzene, etc. Synthetic lubricating oils resulting from polymerization of unsaturated hydrocarbons or other oleaginous materials within the lubricating oil viscosity range such as high molecular weight polyoxyalkylene compounds such as polyalkylene glycols and esters thereof, aliphatic diesters of dicarboxylic acids such as the butyl, hexyl, 2-ethylhexyl, decyl, lauryl, etc., esters of sebacic acid, adipic acid, azelieic acid, etc., may be thickened by the ureido compounds of the present invention to produce excellent greases. Polyfluoro derivatives of organic compounds, particularly hydrocarbons and dibasic acid esters of H(CF<sub>2</sub>)<sub>n</sub>CH<sub>2</sub>OH, in the lubricating oil viscosity range have shown excellent promise when thickened with compounds of the present invention.

Greases of the present invention may be produced by one of the following methods:

(1) The thickener may be prepared apart from and then admixed with the lubricant vehicle and milled in a colloid mill, 3-roll mill, etc.

(2) The thickener may be formed in situ in the oil by introducing the reactants and the desired amount of lubricant vehicle, heating for a relatively short time, e. g. from about five minutes to an hour to complete the reaction, and then cooling and milling the mixture.

(3) As a slight modification of method 2 above, a solvent such as chloroform, ethyl acetate, dioxane, 2-butanone, benzene, etc., may be employed as a diluent and mutual solvent for the reactants. The solvent is then evaporated and the grease is milled, etc., substantially as set forth. Co-pending Swakon and Brannen application for Letters Patent Serial Number 392,996, filed November 18, 1953, now U. S. 2,710,841, is directed to the preparation of substituted urea thickened greases generally by the in situ technique.

(4) As a step in any of the above three methods, it has been found that improved properties may be imparted to the grease by "heat-treating" the grease mixture, i. e. subjecting the same to an elevated temperature for at least about half an hour and preferably longer, e. g. from about 1 to 20 hours. Prolonged heating at such temperature may evaporate a portion of the lubricant vehicle; this loss should be replaced and then the mixture should be milled. The temperature to which the mixture may be heated will, of course, depend upon the particular lubricant vehicle employed. Thus, a silicone polymer oil may be heated to a temperature of about 450° F. but mineral oils, diesters, and other synthetic oils may be heated from about 200° to 400°.

The present invention is illustrated by the following examples:

#### Example I

One-hundredth of mole (1.84 grams) of benzidine, dissolved in ethyl acetate, was added to one-hundredth of mole (2.5 grams) of p,p'-diisocyanato-diphenylmethane in a solvent-extracted SAE 40 petroleum oil (17.4 grams). An immediate reaction occurred which resulted in the thickening of the mixture. The mix was heated and the

solvent removed by distillation. After the solvent was removed, the resultant product was heated to 300° F., stored in an oven at 300° F. for two hours, cooled to about 80° F., and then milled. The finished grease containing 20% of predominantly the polyureido compound was a smooth short-fibred product having a micropenetration<sup>1</sup> of 168.

#### Example II

10 A polyureido thickened solvent extracted SAE 40 petroleum oil was prepared as in Example I, using one-hundredth mole (1.08 grams) of p-phenylene diamine in place of the benzidine. The finished grease product, containing 20% of the polyureido compound was smooth and short-fibred and had a micropenetration of 60.

#### Example III

20 A mixture of one-fiftieth mole (5.0 grams) of p,p'-diisocyanatodiphenylmethane in a solvent extracted SAE 40 petroleum oil and one-hundredth mole each of benzidine (1.84 grams) and p-phenylenediamine (1.08 grams) dissolved in ethyl acetate was heated at 300° F. for about fifteen minutes and the solvent removed by evaporation. The solvent-free product was then stored at 300° F. for 25 two hours, cooled to 80° F., and then milled. The finished grease product containing 20% of the polyureido compound was smooth and short-fibred and had a micropenetration of 78.

The stability of polyureido thickened greases is illustrated by the following micropenetration data on the greases after being held at 300° F. for one, two, and three days.

| Grease                | Micropenetration <sup>1</sup> (after milling) |         |          |            |
|-----------------------|-----------------------------------------------|---------|----------|------------|
|                       | Initial                                       | One Day | Two Days | Three Days |
| Grease of Example I   | 168                                           | 148     | 177      | 153        |
| Grease of Example II  | 60                                            | 87      | 118      | 154        |
| Grease of Example III | 78                                            | 54      | 58       | 60         |

<sup>1</sup> Kaufman, G., Finn, W. J., and Harrington, R. J., Ind. Eng. Chem., Anal. Ed., 11, 108 (1939).

#### Example IV

45 An intimate mixture of DC 550 Silicone Fluid and dry powder from the reaction of bitolyene diisocyanate and water was passed over a three-roll mill. The resulting product is a bright, smooth paste. Penetration data on four greases prepared by this method are:

| Concentration of Thickener, Percent | Penetration<br>1/4-Size<br>Cone <sup>1</sup> |
|-------------------------------------|----------------------------------------------|
| 10                                  | 86                                           |
| 12 <sup>2</sup>                     | 68                                           |
| 15                                  | 62                                           |
| 15                                  | 67                                           |

<sup>1</sup> Proposed ASTM.  
<sup>2</sup> A. B. E. C.-N. L. G. I. bearing tests described in copending application Ser. No. 318,321 (supra) at 450° F. and 10,000 R. P. M. ran 211 and 344 hours.

#### Example V

Grease made by method used in Example IV except diisooctylazelate used in place of DC 550 Silicone Fluid. The resulting grease containing 12.5% thickener had a 1/4-size cone penetration of 63.

#### Example VI

70 Grease made by the method used in Example IV and using a solvent-extracted SAE 40 grade petroleum oil had a 1/4-size penetration of 72 with 15% concentration of thickener.

<sup>1</sup> Kaufman, G., Finn, W. J., and Harrington, R. J., Ind. Eng. Chem., Anal. Ed., 11, 108 (1939).

Greases of the present invention can contain well known additives such as anti-oxidants, oiliness agents, extreme pressure agents, anti-foam agents, etc. without departing from the scope of the invention.

Although the present invention has been described with reference to specific preferred embodiments thereof, the invention is not to be considered as limited thereto, but includes within its scope such modifications and variations as come within the spirit of the appended claims.

I claim:

1. A lubricant grease comprising a lubricant vehicle thickened with from about 2% to about 50%, by weight, of at least one ureido compound having the general formula



wherein Z and Z' are terminal reactive radicals selected from the group consisting of  $-NH_2$  and  $-NCO$  radicals and mixtures thereof, x is an integer 0 to 5, and R, R', and R'' are organic radicals selected from the group consisting of an alkylene radical, a substituted alkylene radical, an arylene radical, a substituted arylene radical and mixtures thereof, said alkylene radical and substituted alkylene radical having 1 to about 30 carbon atoms, and said arylene and substituted arylene radical having no more than 14 cyclic carbon atoms.

2. A lubricant grease as described in claim 1 in which the lubricant is a hydrocarbon lubricating oil.

3. A lubricant grease as described in claim 1 in which the lubricant vehicle is a silicone polymer oil in the lubricating oil viscosity range.

4. A lubricant grease as described in claim 1 in which the lubricant vehicle is an acyclic ester of an aliphatic dicarboxylic acid.

5. A lubricant grease as described in claim 1 in which the lubricant vehicle is a polyfluoro-compound in the lubricating oil viscosity range.

6. A lubricant grease as described in claim 1 in which R, R', and R'' are organic radicals selected from the group consisting of an arylene radical, a substituted arylene radical and mixtures thereof, said arylene and substituted arylene radicals having not more than 14 cyclic carbon atoms.

7. A lubricant grease as described in claim 1 in which R, R', and R'' are organic radicals selected from the group consisting of an alkylene radical, a substituted alkylene radical and mixtures thereof, said alkylene and substituted alkylene radicals containing from 1 to about 30 carbon atoms.

8. A lubricant grease comprising a lubricant vehicle thickened with from about 2% to about 50%, by weight, of at least one polyureido compound having the general formula



in which x is an integer 1 to 5 and R, R', and R'' are organic radicals selected from the group consisting of an alkylene radical, a substituted alkylene radical, an arylene radical, a substituted arylene radical and mixtures thereof, said alkylene radical and substituted alkylene radical having 1 to about 30 carbon atoms, and said arylene and substituted arylene radical having no more than 14 cyclic carbon atoms.

9. A lubricant grease comprising a lubricant vehicle thickened with from about 5% to about 40%, by weight, of a polyureido compound having the formula



15 in which R is a phenylene radical.

10. A lubricant grease comprising a lubricant vehicle thickened with from about 5% to about 40%, by weight, of a polyureido compound having the formula



in which R is a bitolylene radical.

11. A lubricant grease comprising a lubricant vehicle thickened with from about 5% to about 40%, by weight, of a polyureido compound having the formula



30 in which R is a phenylene radical and R' is a biphenylene radical.

12. A lubricant grease comprising a lubricant vehicle thickened with from about 5% to about 40%, by weight, of a polyureido compound having the formula:



13. A lubricant grease comprising a lubricant vehicle thickened with from about 5% to about 40%, by weight, of a polyureido compound having the formula



45 in which Ar represents a phenylene radical.

#### References Cited in the file of this patent

#### UNITED STATES PATENTS

- |    |           |               |       |               |
|----|-----------|---------------|-------|---------------|
| 50 | 2,292,443 | Hanford       | ----- | Aug. 11, 1942 |
|    | 2,710,839 | Swakon et al. | ----- | June 14, 1955 |
|    | 2,710,840 | Swakon et al. | ----- | June 14, 1955 |
|    | 2,710,841 | Swakon et al. | ----- | June 14, 1955 |

U. S. DEPARTMENT OF COMMERCE  
PATENT OFFICE

**CERTIFICATE OF CORRECTION**

Patent No. 2,832,739      Edward A. Swakon      April 29, 1958

It is hereby certified that error appears in the printed specification of the above numbered patent requiring correction and that the said Letters Patent should read as corrected below.

Column 2, line 25, for that portion of the formula reading "(NH-CO-NH-R")" read -- (NH-CO-NH-R"--); column 8, line 27, extreme left-hand portion of the formula, for "H<sub>2</sub>H--" read -- H<sub>2</sub>N- --.

Signed and sealed this 1st day of July 1958.

(SEAL)

Attest:

KARL H. AXLINE

Attesting Officer

ROBERT C. WATSON  
Commissioner of Patents